

## UNITED STATES PATENT OFFICE

2,155,678

## MOTOR FUEL

Johan C. D. Oosterhout, Port Arthur, Tex., assignor to The Texas Company, New York, N. Y., a corporation of Delaware

No Drawing. Application June 25, 1935,  
Serial No. 28,247

9 Claims. (Cl. 44—9)

This invention relates to the stabilization of anti-knock reagents for motor fuels and more particularly to the stabilization of anti-knock reagents of the tetra-ethyl lead type, by the provision in the reagent of a stabilizing agent which will prevent or retard deterioration of the anti-knock material on storage.

It is customary to add to commercial gasolines, especially those of high anti-knock value, an anti-knock reagent to increase or maintain the anti-knock property. One of the most common reagents is tetra-ethyl lead, although other metallo-organic compounds, such as metal carbonyls, particularly nickel carbonyl, are sometimes used. The anti-knock compounds are often added to gasolines in the form of prepared reagents of a predetermined composition which are easily handled, distributed and dissolved in the gasoline to be treated. It is desirable that these reagents be stable and not decompose or deteriorate on storage or handling, and even after they are incorporated into the gasoline.

The present invention is directed particularly to the treatment of a tetra-ethyl lead type of anti-knock reagent. This reagent is commonly provided in the form of a fluid composition which may be readily dissolved in the gasoline in any desired proportions. A typical composition of this type, commonly known in the trade as "Ethyl Fluid", is as follows:

|                     | Per cent by weight |
|---------------------|--------------------|
| Tetra-ethyl lead    | 61.69              |
| Ethylene dibromide  | 25.09              |
| Ethylene dichloride | 8.50               |
| Dye                 | 0.12               |
| Kerosene            | 3.66               |
| Undetermined        | 0.94               |

Such tetra-ethyl lead compositions or ethyl fluids have the tendency to decompose and deteriorate on storage. It is not uncommon to find a sediment or precipitate in the bottom of drums or containers in which the material has been stored or transported. The decomposition, furthermore, is often more rapid in sunlight or diffused light than in the dark. When the reagent, which is partially decomposed, is added to gasoline it is necessary to use care that none of the precipitate is transferred to the gasoline, since a cloudy appearance will be imparted thereto. Although the gasoline to which the anti-knock reagent is added be clear and free from any cloud, after the antiknock reagent is added the reagent often decomposes in the gasoline,

whereby a cloud or even a precipitate may form in the gasoline as the result of the decomposition of the reagent.

I have found that a tetra-ethyl lead anti-knock reagent or ethyl fluid may be stabilized by the addition thereto of a small proportion of lecithin, such as produced from soy beans. A crude or purified product may be used but I prefer a purified product relatively free from fatty oils. Crude phosphatides may also be used. The quantity to be added may vary within rather wide limits and various quantities between about 1-15% are satisfactory. It is ordinarily not necessary to use over about 10%. The following table shows the periods of stabilization of a sample of ethyl fluid by certain quantities of lecithin:

| Quantity of lecithin | Stabilization period in dark |
|----------------------|------------------------------|
| None                 | 20                           |
| 1%                   | 3 to 4 days.                 |
| 7%                   | Several weeks.               |
| 8%                   | 12 months.                   |
| 10%                  | 15 months.                   |
|                      | Indefinite.                  |

The anti-knock reagent containing lecithin in addition to being stable itself on storage also has the advantage of stabilizing the gasoline to which it is added. The gasolines to which ordinary ethyl fluid has been added have been found to become cloudy or form a precipitate, particularly in sunlight, whereas gasolines containing ethyl fluid stabilized by lecithin remain unchanged for long periods of time. The invention has the further advantage that the corrosion of tanks or other containers containing ethyl fluid which has been stabilized as herein described, is substantially prevented.

The subject matter of this application is related to that in a co-pending application, Serial No. 748,076, of Harry V. Rees and Johan C. D. Oosterhout, filed October 12, 1934, which has to do with the stabilization of gasolines containing tetra-ethyl lead anti-knock reagents by means of combinations of lecithin and certain gum inhibitors.

Obviously many modifications and variations of the invention, as hereinbefore set forth, may be made without departing from the spirit and scope thereof, and therefore only such limitations should be imposed as are indicated in the appended claims.

I claim:

1. A composition comprising tetraethyl lead normally unstable and tending to deteriorate and

form a cloud, stabilized against such deterioration and cloud formation by lecithin in the amount of about 1 to 15% of the weight of the tetraethyl lead, said tetraethyl lead being the sole essential ingredient stabilized by said lecithin.

5 2. A composition comprising gasoline, tetraethyl lead and lecithin, said gasoline being normally gum stable and substantially unaffected in gumming tendency by the tetraethyl lead, said tetraethyl lead being normally unstable and tending to deteriorate and form a cloud, and said lecithin being present in an amount of about 1 to 15% of the weight of the tetraethyl lead and substantially preventing said deterioration and cloud formation.

10 3. A process for the stabilization of a composition containing tetraethyl lead against deterioration on storage, said composition otherwise substantially stable except for the tetraethyl lead, which comprises adding to the composition lecithin in the amount of about 1 to 15% of the weight of the tetraethyl lead.

15 4. A process for the stabilization of gasoline containing tetraethyl lead, said gasoline otherwise

substantially stable except for the tetraethyl lead which tends to deteriorate and form a cloud, comprising adding to the gasoline lecithin in the amount of about 1 to 15% of the weight of the tetraethyl lead.

5 5. A process for producing a stable tetraethyl lead composition which comprises mixing with tetraethyl lead a small amount of a phosphatide.

6. A process for producing a stable tetraethyl lead composition which comprises adding to ethyl fluid a small amount of a lecithin-containing compound.

10 7. A process for producing a stable tetraethyl lead composition which comprises adding lecithin to ethyl fluid in sufficient amount to substantially retard deterioration thereof on storage.

15 8. A tetraethyl lead antiknock reagent, normally tending to deteriorate on storage, and containing lecithin in sufficient amount to retard such deterioration.

20 9. A fluid antiknock reagent, comprising tetraethyl lead and 1-15% of lecithin.

JOHAN C. D. OOSTERHOUT.